

## UNITED STATES PATENT OFFICE

JOHN A. HAMMOND, OF ALBANY, CALIFORNIA, ASSIGNOR TO CALIFORNIA CAP COMPANY, OF OAKLAND, CALIFORNIA, A CORPORATION OF CALIFORNIA

## EXPLOSIVE

No Drawing.

Application filed July 7, 1930. Serial No. 466,043.

This invention relates to explosives, and particularly to a treatment of black powder, and has for its objects a process whereby the powder is rendered slow burning while at the same time retaining its granular and free pouring characteristics so that it may be handled in conventional apparatus for filling fuses.

Other objects of the invention will appear in the following description.

It has long been desirable to slow down the burning speed of various powders used for fuse making so as to get the required delay without an extremely long fuse which is objectionable for several reasons besides greatly increasing the danger of failure, and many prior attempts have been made to treat fuse powders both for slowing their burning speeds as well as to partially waterproof them, or prevent spontaneous or slow decomposition. Such prior treatments have included admixing various slower burning powders or retarding substances with the fuse powder, also incorporating therewith oils, greases, paraffine etc. to form a mass more or less moisture proof and of slower burning properties than the plain powder.

It has also been found that various gums, resins and pitches including asphaltum could be mixed as a dry powder, or melted into the powder or with the sulphur content powdered and admixed. Also various varnishes have been incorporated in black powder and other fuse powders in an attempt to control the explosive or burning properties thereof.

However, while these earlier methods all effected certain improvements in the properties of the powders, the requirements of their day were not at all the requirements of today when successive delay fuses are an article of automatic manufacture and must be absolutely relied upon to set off a series of blasts in the order of the fuse numbers or delay indicia, and to do this every time under every condition of use.

Also since there is a tendency of the art to move toward the adoption of an all metal delay fuse of much shorter length than the old type fuses, and wherein the powder, of

definite quantity, is compacted under definite pressure in the bores of metal fuse tubes, it becomes a matter of vital importance that the time control and absolute homogeneity of the powder used be at all times absolutely constant. This is especially true with all metal delay fuses as shown and described in my copending patent for blasting caps filed under Serial No. 438,304 on March 24, 1930, for in the manufacture of such fuses the powder must be absolutely uniform in its properties from end to end of the bore, and should also be free running for proper handling in the filling and compacting apparatus.

With the above requirements in mind it will be seen that a powder treated with a sticky varnish could not be handled, and if permitted to dry and then broken up would present irregularly agglutinated grains, also of uneven burning properties on account of the settling of the varnish to the lower strata of the mass. Several of the dry mixes were found fairly good but much too rapid in burning speed or too erratic if more inert material were added.

After long experimentation I have found the proper substance and the proper mode of treating black powder or other fuse powders whereby a perfectly homogeneous evenly retarded, free pouring, damp-proofed and absolutely dependable powder for metal fuses may be produced, and a great many actual tests of metal delay fuses made with the powder, extending over a period of time, have not shown a single failure.

To prepare a fuse powder in accordance with my process I take a quantity of any fuse powder such as black powder, saturate it with a solution of a certain grade of asphaltum carried in a highly volatile solvent, and at once triturate the mass until the solvent has evaporated to leave the powder granules dry and each coated on all sides with the asphaltum. The grade of asphaltum is one which will be free from stickiness, and the solvent should be one which will not act to dissolve out the sulphur content of the powder or else highly volatile so that it may be gotten rid of before any ob-

jectional action on the sulphur has taken place.

As an example I prepare a solution in the proportion of asphaltum 40 grams to 250 c. c. of carbon bisulphide. The grade of asphaltum having a penetration test of 0 to 10 and preferably what is known as air blown.

I next add to a weighed quantity of black powder, placed in a suitable receptacle, say 10 6 ounces, 80 c. c. of the above asphaltum solution. This will be found to just "saturnate" or rather fill the interstices of the mass, and as soon as the solution has percolated to the bottom of the powder it is triturated in 15 suitable non-sparking apparatus, preferably under the influence of any suitable exhaust apparatus to remove the vapors of the bisulphide, until the powder is dry, a matter of a few moments.

20 The powder so treated will be found to carry about 8% of asphaltum to the weight of the untreated powder, to be free pouring and with each granule completely surrounded or enclosed in a film of the hard asphaltum. Tho if the process has not been perfectly carried out or any slight agglutination should manifest itself the powder may be passed through a suitable screen to insure absolute uniformity and separate any undesirable large grains.

Instead of the solvent above mentioned I have also secured good results with carbon tetrachloride, also benzole, and I have used 25 other grades of asphalt both softer and harder including gilsonite but I have found the grade and solvent mentioned satisfactory in every respect.

The above treatment yields a powder which 30 when confined in a metal fuse will burn at about one foot in 144 seconds, tho for still slower burning it suffices to increase the density of the asphaltic solution.

By the above process of using a definite 35 quantity of a known density of asphaltum solution on a unit quantity of powder and triturating same until dry and said definite quantity of asphaltum has evenly coated the grains of the unit quantity of powder it is 40 possible to obtain a uniform product without variance, as required for modern delay fuse production, and which I believe represents a valuable and new step forward in the art. I therefore claim:

45 1. The method of treating black powder which comprises mixing the powder with a solution of asphaltum carried in a volatile solvent and triturating the mass until a substantially dry free flowing powder results 50 each granule of which is coated exteriorly with the asphaltum.

2. The method of treating black powder 55 which comprises mixing the powder with a solution of hard asphaltum dissolved in carbon bisulphide and triturating the mass until a substantially dry powder results.

3. The method of treating black powder which comprises mixing the powder with a solution of asphaltum of from 0 to 10 penetration dissolved in carbon bisulphide and 60 triturating the mass until a substantially dry 70 powder results.

4. The method of treating black powder which comprises mixing the powder with a solution of hard asphaltum dissolved in carbon bisulphide and triturating the mass until 75 a substantially dry powder results, carrying on the exterior of its granules about eight per centum of asphaltum by weight to the weight of untreated powder.

5. An explosive comprising black powder, 80 the individual grains of which carry an enveloping coat of hard asphaltum non-adhesive at ordinary temperatures, whereby the powder is free flowing.

6. An explosive comprising black powder, 85 the individual grains of which carry an enveloping coat of hard asphaltum non-adhesive at ordinary temperatures, and in quantity equal to about 8% of the weight of the untreated powder, whereby the powder 90 is free flowing.

JOHN A. HAMMOND.

95

100

105

110

115

120

125

130